

[54] **SOAP THICKENED HYDRAULIC OIL COMPOSITION**

[75] Inventors: **John Q. Griffith, III; Edward S. Williams, both of Claymont, Del.; William H. Reiland, Jr., West Chester, Pa.**

[73] Assignee: **Sun Oil Company of Pennsylvania, Philadelphia, Pa.**

[\*] Notice: The portion of the term of this patent subsequent to Sept. 26, 1989, has been disclaimed.

[22] Filed: **Sept. 7, 1971**

[21] Appl. No.: **178,479**

**Related U.S. Application Data**

[63] Continuation-in-part of Ser. No. 34,899, May 5, 1970, Pat. No. 3,694,363.

[52] **U.S. Cl.** ..... **252/72, 252/35, 252/41, 252/73, 252/74, 252/75, 252/76**

[51] **Int. Cl.** ..... **C09k 3/00**

[58] **Field of Search** ..... **252/72-76, 252/35, 41; 208/14, 18**

[56] **References Cited**

**UNITED STATES PATENTS**

|           |         |                |          |
|-----------|---------|----------------|----------|
| 2,528,348 | 10/1950 | Denison et al. | 252/75   |
| 3,039,967 | 6/1962  | Henry et al.   | 252/75   |
| 3,156,652 | 11/1964 | Fuehr          | 252/75   |
| 3,175,976 | 3/1965  | Fuehr          | 252/75   |
| 3,203,896 | 8/1965  | Latos et al.   | 252/75 X |
| 3,242,068 | 3/1966  | Paterson       | 208/18 X |

|           |         |                 |          |
|-----------|---------|-----------------|----------|
| 3,284,340 | 11/1966 | Halik et al.    | 208/18 X |
| 3,383,312 | 5/1968  | Coppock         | 252/35 X |
| 3,498,920 | 3/1970  | Nichols et al.  | 252/73 X |
| 3,533,952 | 10/1970 | Pruitt et al.   | 252/73 X |
| 3,544,472 | 12/1970 | Bray et al.     | 252/73   |
| 3,663,427 | 5/1972  | Thomas et al.   | 208/18 X |
| 3,682,813 | 8/1972  | Dun et al.      | 208/18 X |
| 3,684,684 | 8/1972  | Coleman et al.  | 208/18 X |
| 3,694,363 | 9/1972  | Griffith et al. | 252/72   |

**OTHER PUBLICATIONS**

Georgi: "Motor Oils and Engine Lubrication," (1950), pub. by Reinhold Pub. Co., pp. 108, 153, 154.

*Primary Examiner*—Leon D. Rosdol

*Assistant Examiner*—Harris A. Pitlick

*Attorney, Agent, or Firm*—G. L. Church, Esq.; J. E. Hess, Esq.; B. A. Bisson, Esq.

[57] **ABSTRACT**

An improved antileak hydraulic oil of the gel-thickened type comprises an effective amount of a lithium soap (e.g., 0.1-1% Li stearate) or an aluminum soap (e.g., 0.5-2% Al stearate), or mixtures of such soaps, and a base oil having a viscosity in the range of 70-3000 SUS at 100°F., said base oil comprising at least one hydro-refined naphthenic oil or a hydrocracked paraffinic oil having a viscosity in the range of 40-12,000 SUS at 100°F. The hydraulic oil can also contain an antirust agent (e.g., 0.02-2%) barium petroleum sulfonate, an antioxidant (e.g., an amine type) and an antiwear (e.g., 0.1-5% zinc dialkyl dithiophosphate).

**18 Claims, No Drawings**

## SOAP THICKENED HYDRAULIC OIL COMPOSITION

### CROSS REFERENCE TO RELATED APPLICATIONS

This application is a continuation-in-part of our application Ser. No. 34,899, filed May 5, 1970, now U.S. Pat. No. 3,694,363 issued Sept. 26, 1972.

The following patents and applications, all assigned to The Sun Oil Company (as is the present application), are related to the disclosure of the present application in that they disclose methods of obtaining aromatic extracts or concentrates, distillate oils, hydrocracked oils and hydrorefined oils, which can be used to make the hydraulic oil composition of the present invention.

The disclosure of all of the following applications and patents is hereby incorporated in the present application:

U.S. Pat. No. 3,462,358 issued 8-19-69, U.S. Pat. No. 3,681,279 issued 8-1-72, U.S. Pat. No. 3,502,567 issued 3-24-70, Ser. No. 730,999 filed 5-22-68, U.S. Pat. No. 3,619,414 issued 11-9-71, Ser. Nos. 850,716 and 850,717 both filed 8-18-69 (both now abandoned), U.S. Pat. No. 3,654,127 issued 4-4-72, Ser. No. issued 8-1-72, Ser. No. 35,231 filed 5-6-70, Ser. No. 60,642 filed 8-2-70 (now abandoned), U.S. Pat. No. 3,715,302 issued 2-6-73, U.S. Pat. No. 3,732,154, issued 5-8-73, U.S. Pat. No. 3,663,427 issued 5-16-72, U.S. Pat. No. 3,666,657 issued 5-30-72, Ser. No. 140,398 filed 5-5-71 and U.S. Pat. No. 3,759,817 issued 9-18-73.

U.S. Pat. No. 3,383,312 to Walter J. Coppock is also pertinent since it describes a method of preparing a fluid soap thickened mineral oil lubricant composition, which method can be useful in practice of the present invention.

### BACKGROUND OF THE INVENTION

The industrial oil market is continuing to grow at a rapid pace. Accompanying this growth is the demand for better lubricant properties. Specific improvements are needed to cope with trends towards more severe operating conditions and better pollution control. In the response to these requirements, research has made important advances in upgrading antiwear and antileak properties. Wear-resistant oils can alleviate the equipment problems and failures caused by increased pressures and temperatures, shock loading, reduced tolerances, etc. Antileak oils can decrease the undesirable loss of lubricants. Not only do these latter oils reduce consumption, but they help curb the pollution of our natural waters. These problems are considered in greater detail in our patent U.S. Pat. No. 3,694,363, issued 9-26-72.

### SUMMARY OF THE INVENTION

An improved antileak hydraulic oil of the gel-thickened type comprises an effective amount of a lithium soap (e.g., 0.1-1% Li stearate) or an aluminum soap (e.g., 0.5-2% Al stearate), or mixtures of such soaps, and a base oil having a viscosity in the range of 70-3000 SUS at 100°F., said base oil comprising at least one hydrorefined naphthenic oil or a hydrocracked oil having a viscosity in the range of 40-12,000 SUS at 100°F. The hydraulic oil can also contain one or more of the following: an antirust agent (e.g., 0.02-2% typically 0.2% barium petroleum sulfonate),

an antioxidant (e.g., 0.05-1% of an amine type), an antifoam (e.g., 0.05-1% of a silicone type) and an antiwear (e.g., 0.1-5%, typically 0.3-2%, zinc dialkyl dithiophosphate, such as zinc-isopropyl, decyldithiophosphate) or tricresylphosphate. For systems having seals comprising synthetic rubbers (e.g., "Buna N", GRS, ABS) it is preferred that the aniline point of the base oil be in the range of 150°-170°F. For systems where the seals are of other rubbers or materials, a higher aniline point may be required (e.g., for the silicone rubbers an aniline point of about 200°F. imparts the proper seal-swelling character to the hydraulic oil). In calculation of the aniline point of the base oil, one must consider the contribution of aromatic additives (e.g., those marketed as seal swell agents) and the hydrocarbon diluent used in many commercial additives. The term "base oil" in the present application refers to the total hydrocarbons of the 40-12,000 SUS viscosity range which are present in the final hydraulic oil, it being understood that some of these hydrocarbons can be contributed via the usual commercial additives.

A preferred antioxidant is DBPC (ditiarybutyl paracresol) or an amine type, used in combination with sufficient zinc dialkyl dithiophosphate to impart antiwear properties (e.g., 0.010-0.020% Zn).

The hydraulic oil can show good antiwear and antileak performance and good hydrolytic and oxidation stability in the ASTM D-943 turbine oil stability test (TOST).

The base oils preferably contain less than 80 ppm of basic nitrogen and can be those described in the previously cited applications of Mills et al. and, more preferably, are blends of two or more hydrorefined naphthenic oils (e.g., a blend of a 100 SUS at 100°F. hydrorefined naphthenic oil and a 2500 SUS at 100°F. hydrorefined naphthenic oil) or a blend of hydrorefined naphthenic oil and hydrocracked paraffinic oil.

In the hydraulic oil of the present invention, leakage reduction is achieved by designing into the lubricant the ability to maintain good rubber seal condition (e.g., by proper choice of aniline point of the base oil) and the ability to obstruct small leaks with retardant materials (e.g., Li or Al soaps or polymers). Plant trials have been conducted comparing the performance of the antileak hydraulic oils of the present invention to current, standard products. Lubricant loss was lowered as much as 88% by the leak resistant formulations. These antileak hydraulic oils of the present invention also have good overall properties and have performed well in many types of plant equipment.

### FURTHER DESCRIPTION

The hydrocarbon base oil can also contain a low nitrogen content paraffinic distillate or solvent raffinate oil, a hydrorefined paraffinic distillate or raffinate, a viscosity index improver (e.g., high molecular weight polybutene or a polyacrylate or polymethylacrylate, preferably the dispersant type), a polycyclic aromatic concentrate (such as cycle stock) or extract (such as a furfural extract from a naphthenic distillate) to adjust the 335 UVA of the base stock (which preferably is in the range of 0.01-0.4, more preferred 0.02-0.2) and/or the aniline point and an unhydrorefined naphthenic distillate or a naphthenic acid-free naphthenic distillate (to improve the D-943 test performance).

Paraffinic oils are those having a viscosity-gravity constant (VGC) in the range of 0.790 to 0.819 (preferably above 0.799).

Naphthenic oils have a VGC in the range of 0.820 to 0.899 and the preferred hydrorefined naphthenic oils have a VGC in the range of 0.840 to 0.899. Hydrorefined, relatively aromatic oils, having a VGC in the range of 0.900 to 0.920, can sometimes be used as a whole or partial substitute for the hydrorefined naphthenic lube. Aromatic oils (including hydrorefined or hydroaromaticized oils) having a VGC in the range of 0.921 to 1.050 and greater, can be useful in minor proportions (e.g., 1-20%) for adjusting the aniline point of the base oil, particularly when the base oil contains a high proportion of a high VI hydrocracked paraffinic oil.

As an additional component, or as a partial or complete substitute for the hydrorefined naphthenic oils previously described, hydraulic oils of the gel or polymer thickened types can contain a wax-free, hydrogenated polyolefin oil (e.g., see Canadian Patent 842,290; U.S. Pat. No. 3,598,740) or a high viscosity index, hydrocracked oil or a mixture of such components. In such blends an aromatic oil or concentrate rich in aromatic hydrocarbons (e.g., cycle oil) may have to be added to obtain the proper aniline point for seal swelling.

The preferred polyolefin oils are polymers or copolymers of  $C_2-C_8$  olefin which have a pour point no greater than  $-35^{\circ}\text{F}$ , and preferably below  $-50^{\circ}\text{F}$ . The hydrogenation can be from 50% to 100% of saturation and, preferably, is to a bromine number no greater than 10, more preferably less than 5. Preferred polyolefins include ethylene-propylene copolymer, polypropylene, polybutene (especially polyisobutylene), and poly(1-octene).

The high VI hydrocracked paraffinic oil component can be obtained by hydrocracking a high viscosity distillate or dewaxed distillate from a paraffinic crude (such as Lagomedio) and typically has a VI in the range of 90-105 and contains in the range of 3-30% of aromatics by clay-gel analysis. The hydrocracked lubes are preferably stabilized (against UV light degradation and sludging) by extraction of the hydrocracked oil with aromatic selective solvents, such as furfural or phenol or by hydrorefining to reduce the 260 UVA at least 30% (preferably 40%).

The preferred "stabilized" hydrocracked oils (whether extracted or hydrorefined) are characterized by having a D-943 test life (to an increase in acid number of 2.0) which is at least 20% lower than the D-943 life of an unstabilized hydrocracked oil but which is at least 20% greater than the D-943 life (with the usual amount of inhibitor) of an unhydrocracked solvent refined lube of the same viscosity.

One process for preparing a high VI hydrocracked oil comprises fractionating the stock material (such as an atmospheric residuum from Lagomedio crude) into three fractions, boiling at (a) from  $720^{\circ}-855^{\circ}\text{F}$ , (b)  $855^{\circ}-980^{\circ}\text{F}$ , and (c) the residuum or a fraction boiling at from  $986^{\circ}-1070^{\circ}\text{F}$ , solvent extracting fraction (b) with a solvent having preferential solubility for aromatics such as furfural, recombining the three fractions, dewaxing to  $0^{\circ}\text{F}$ . pour point or lower, and hydrocracking the combined fractions at from  $720^{\circ}-800^{\circ}\text{F}$ . using a hydrogen partial pressure of from 2,000 to 3,000 psi, and a sulfided nickel-tungsten catalyst supported on

silica-alumina and containing a minor amount of a fluoride (e.g., Gulf GC-6). The higher boiling fraction is deasphalted if required.

Examples of such hydrocracked oils are found in U.S. Pat. No. 3,579,435 and in the following commonly-owned applications (the disclosure of which is incorporated herein by reference):

| 10 | Serial No. | Filing Date | Inventor(s)     |
|----|------------|-------------|-----------------|
|    | 780,241    | 11-19-68    | Thompson et al. |
|    | 875,502    | 11-10-69    | Thompson        |
|    | 64,656     | 8-17-70     | Kress           |

15 The preferred amount of gelling agent to add to a given base oil can be determined from an experimentally obtained "soap in oil curve." That is, various amounts of soap are added to base oil samples (which can also include some or all of the other additives) and the viscosity of the soap-oil samples is determined. The results are plotted as a viscosity versus concentration curve. In such a curve, a point will be found where the viscosity suddenly increases greatly. This will be the minimum concentration of soap which should be put into the oil for antileak protection. Generally, about 0.1% more soap than this minimum concentration should be put into the oil. The maximum amount of soap (or other gelling agent) will be where the solution "lumps-up" or becomes non-homogeneous.

20 30 The preferred soaps are lithium or aluminum stearate; however, any of the prior art lithium or aluminum soaps which have been used in petroleum lubricants can be useful in hydraulic oils of the present invention. Such soaps are shown, for example, in U.S. Pat. Nos.

25 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 94

For other rubbers, such as the silicones, a different aniline point range may be required for proper swelling (e.g., for silicone rubbers an aniline point in the range of 195°-215°F. is preferred).

Note that such prior art as U.S. Pat. No. 2,408,983 (which at column 5 shows an aniline point of 178°F.), U.S. Pat. No. 2,489,300 (which in examples) and 2 shows aniline points of 145°F. and 131°F.) and U.S. Pat. No. 2,616,854 (which shows a range of 175°-190°F.) lead the art away from our preferred ranges of 150°-170°F. and 195°-215°F.

Besides utilizing a base oil which properly conditions the rubber seals and gaskets, leakage can also be reduced by restricting small openings with leak retardant materials. The leak retardant must be carefully selected so that the properties of the lubricant are not harmed. There are two basic types of antileak additives presently being used. The first is the polymeric type which includes material having molecular weights greater than several hundred thousand (e.g. polybutene). The second involves gelling agents (e.g., organic salts of polyvalent metals or "soaps") which can have molecular weights of about three hundred.

It has been postulated that the polymeric materials develop a more rigid structure in areas of low shear rates, such as the threads of a leaky coupling. The viscosity, therefore, increases and flow is hindered from the high pressure zone.

Gelling agents are believed to perform in a different manner. That is, they build up fibers or log jams in small openings, thereby barricading them and preventing fluid flow.

Both of these types of antileak additives shear down temporarily when subjected to pump, valve, etc. operations. Permanent shear loss is also experienced to a limited degree. Because this does occur, the equipment is able to operate satisfactorily without clogging problems.

There are no known products which completely stop leakage. One reason for this is that the types of leak retardants which can be used are limited by other performance characteristics. The antileak component must be a material which will not cause plugging in filters as small as 5 microns or interfere with servovalve operation where clearances are extremely critical. Other properties of the lubricant itself, such as the oxidation stability, foam resistance, etc., must not be sacrificed.

In the following examples, as in the rest of this application, all percentages are by weight.

#### ILLUSTRATIVE EXAMPLES

The best way to evaluate new formulations is in the actual machinery in which leak problems are encountered. There is presently no standard way to measure antileak properties in the laboratory. A laboratory method has been devised, however, which appears to correlate with field experience. This test has been useful in measuring good versus bad antileak oils or improvements over a given reference oil. The reference oil can be, for example, a rust and oxidation (R&O) inhibited paraffinic hydraulic oil. This R&O reference contains all of the necessary additives to guarantee good lubricant performance but incorporates no leak retardants.

The apparatus in which leakage characteristics are measured is a U-shaped combination of  $\frac{3}{4}$ " iron nip-

les, union sleeves, and elbows. They are joined together by hand tightening in a U-shape and then spot welded to hold in a fixed position. One end of the U is capped, the other end is connected to a pressure source. The procedure utilizes a 300 cc oil sample. The system is pressurized to 30 psi. with nitrogen and allowed to stand for 1 hour. The oil which has dripped out at the end of this period is collected and weighed.

As with most screening tests, this method can only predict whether the oil is better than another. It cannot indicate the degree of improvement to be provided. Nothing but a large amount of field experience can supply this information.

#### EXAMPLE I

##### Polymeric Type Antileak Hydraulic Oils

The incorporation of proper polymers into hydraulic oils are concentrations as high as 5% can provide leakage protection. As can be seen in Table I, a typical product containing a high molecular weight butene polymer also has good overall properties. The base oils, which are naphthenic in nature, have an aniline point of 152°F. and generally provide good rubber seal conditioning. Water separation, foam resistance, rust protection are all acceptable. The oxidation stability, as measured by the ASTM D-943 procedure, is 1,250 hours. Leakage resistance, according to the laboratory test is approximately 41% less than that of a normal R&O hydraulic oil.

Two field trials were run with the polymeric antileak hydraulic oil. The results of these equipment evaluations are listed in Table II. In the first field trial listed, three broaches were run for a period of two months at each of three separate plant locations. The broaches were first run with the R&O hydraulic oil to determine baseline data. The polymeric antileak oil was then added to these same machines and consumption characteristics measured. As can be seen, the three divisions reported improvements of 46%, 88% and 50%, respectively. The second trial listed in Table II was run on a total plant basis. All machines using R&O hydraulic oil were studied for consumption during a 6 month period. These same machines were then charged with the polymeric antileak hydraulic oil for an equivalent 6 month period. After the one year trial, this plant measured a reduction in lubricant consumption of 28%. Table III lists 12 machines in the second plant trial which had the largest amount of leakage with the R&O type hydraulic oil. The machines covered a wide range of operations. In these pieces of equipment, the leakage reduction afforded by the polymeric antileak hydraulic oil was 39%, significantly more than the percentage reported for the total plant. Good leakage reduction is obtained with 1-6% polybutene (typically 2%).

The polymeric antileak lubricant after the field trials had experienced only the normal amount of degradation. Filter and valve operations were completely satisfactory. The one final property which had changed more than that of the R&O hydraulic oil was viscosity. The polymer loss by sheardown caused a viscosity decrease of approximately 10%. This loss did not cause any performance problems.

A polymer thickened antileak oil with good performance in the D-943 test comprises 2% of a polybutene additive, 0.6% DBPC, 0.7% zinc dialkyl dithiophosphate and the remainder a blend of hydrorefined naph-

thenic oil and hydrocracked paraffinic oil, the blend having an aniline point of 200°F. and a viscosity at 100°F. of 300 SUS.

#### EXAMPLE II

##### Gel Type Antileak Hydraulic Oils

An antileak hydraulic oil was compounded using lithium stearate as a gel type leak retardant.

The gel type antileak hydraulic oil composition had a SUS viscosity of about 250 at 100°F. and was prepared from a 200 SUS (at 100°F.) base oil containing 56 ppm of basic nitrogen and obtained by blending 25% of 2400 SUS (at 100°F.) hydrorefined naphthenic oil and 75% of 100 SUS (at 100°F.) hydrorefined naphthenic oil. Both hydrorefined naphthenic oils were obtained from naphthenic acid-free naphthenic distillate by hydrogenation at 625°F., 1200 psig, of 80% hydrogen, 0.2 LHSV with a presulfided Ni-Mo-oxide catalyst. In addition to the base oil, the hydraulic oil contained 0.25% Li stearate, 0.17% of an amine type antioxidant (Dupont Ortholeum), 10 ppm of a defoamer (Dow Corning Silicone), 0.2% of a neutral barium petroleum sulfonate antirust agent, and 0.7% Zn dialkyl dithiophosphate (Elco 114). The Zn dialkyl dithiophosphate imparts especially useful antiwear and antioxidant properties to the hydraulic fluid and has excellent hydrolytic stability. The alkyl group of this additive can vary considerably, depending on the manufacturer; however, all such presently commercially available Zn dialkyl dithiophosphate antiwear additives can be used in the fluids of the present invention.

Specific gelling agents (e.g., Li or Al soaps) appear to be more efficient than the polymers in reducing leakage at concentrations up to 3%. The Al soaps are less hydrolytically stable than the Li soaps. Lubricants containing these materials are, however, also somewhat less stable to oxidation. The overall properties of the gel thickened hydraulic oil are good. A hydrogenated naphthenic type blended base oil with an aniline point of 160°F., for example, can be used to provide seal swell. Oxidation stability, as measured by the ASTM D-943 procedure, is about 300 hours less than the polymeric version but about 200% better than a comparable oil containing naphthenic acid-free naphthenic distillate instead of the hydrorefined oil. The leak resistance of the gel type oil made from the hydrorefined base stock is twice as good as measured in laboratory equipment.

Field trial data was obtained with the gel antileak hydraulic oil of this example. Three presses were tested, one a horizontal type, and the other two vertical. These presses were operated from 880 hours to 1,944 hours. Leakage reduction when compared to the R&O hydraulic oil was 55%, 85% and 60%, respectively. These values are higher than the reductions reported for the polymeric antileak hydraulic oil. Filter and valve performance were completely acceptable. After this trial the condition of the product was excellent. There was not significant viscosity or acid buildup. A viscosity loss of about 15% occurred due to the sheardown of the gel, but there was still enough of the leak retardant present to maintain good leakage reduction.

Actual equipment testing has shown that polymeric antileak hydraulic oils can reduce losses by 23 to 88%. The gel containing antileak hydraulic oils are more efficient with reductions of 55 to 85% in plant equipment.

#### EXAMPLE III

An antileak hydraulic oil was compounded using the same blended (i.e., 100 SUS and 2400 SUS hydrorefined naphthenic oils) base oil as in Example II; however, the additives were different from those in Example II, namely, 0.7% tertiarybutyl para cresol (DBPC), 0.05% alkyl (C<sub>8</sub>–C<sub>18</sub>) substituted succinic acid (Lubrizol 850), 0.1% dioctyl dithio-thia-diazole (Amoco 150), 2 ppm silicone defoamer (1000 cSt at 100°F., Dow Corning 200 fluid). This hydraulic oil required about 1000 hours of ASTM D-943 testing to reach an acid number end point of 2.0. In contrast, a hydraulic fluid with the same additives but made from unhydrorefined naphthenic oil failed after 200 hours of D-943 testing.

Addition of zinc dialkyl dithiophosphate to provide 0.015% Zn in the final compounded oil imparts good antiwear properties.

#### EXAMPLE IV

Two antileak hydraulic oils were compounded using the additives in Example III (that is, one oil contained zinc dialkyl dithiophosphate) and as the base oil a 200 SUS blend of a 100 SUS hydrocracked paraffinic lube and a 500 SUS hydrocracked paraffinic lube. Both oils showed better D-943 test performance than the corresponding oils containing hydrorefined or unhydrorefined base oils.

#### EXAMPLE V

An antileak hydraulic oil was compounded using the same amount of lithium stearate and the same base oil as in Example I. The addition of 5% of a 200 SUS "Duo-Sol" extracted paraffinic lube having an aniline point of 226°F. improved the D-943 performance of the hydraulic oil. Similar results were obtained with 5% of a 152°F. aniline point blend of 25% 100 SUS and 75% 2500 SUS naphthenic acid-free naphthenic distillates or with 2½% of the paraffinic oil and 2½% of the naphthenic oil blend.

A 200 SUS hydrocracked paraffinic lube can be used instead of the paraffinic lube in this example.

The attached Table VI lists the properties of a series of hydrocracked oils (stabilized by solvent extraction) which are especially suitable components for blending with hydrogenated and/or unhydrogenated naphthenic oils and/or an aromatic concentrate to provide a suitable base stock having an aniline point in the range of 150°–170°F. For such blending, the following formula can be used to predict the aniline point (AP) of the blended base stock (AP Base):

$$\text{AP Base} = (X) (\text{AP Paraffinic Component}) + (1-X) (\text{AP Naphthenic Component})$$

where X is the volume fraction of the paraffinic component and 1-X is the volume fraction of the naphthenic component.

An especially useful blended paraffinic component is obtained by blending 90 parts by volume of a 60 SUS at 100°F. hydrocracked paraffinic oil with 10 parts by volume of the unhydrorefined paraffinic oil (obtained by Duo-Sol extraction of a paraffinic distillate).

Another paraffinic component, which can also be used as a textile process oil (due, in part, to its high unsulfonatable residue) is obtained by substitution of the hydrocracked paraffinic oil for the solvent refined oil. Similar paraffinic components of higher viscosity and

differing aniline points can be obtained by blending other hydrorefined and unhydrorefined paraffinic lube stocks of higher viscosity.

Some commercial additive packages contain aromatic compounds. The contribution of these aromatics to the aniline point of the base oil must be considered in calculations.

When the base oil contains a hydrocracked oil component, satisfactory seal swelling can be obtained at higher aniline points (e.g., about 200°F.).

An especially useful soap and polymer thickened oil, for lubrication of textile machinery, can be made by adding lithium stearate (or lithium palmitate, laurate, oleate, etc.) and high molecular weight polyisobutylene to a hydrogenated naphthenic oil having a viscosity in the range of 60-300 SUS at 100°F. For example, sufficient lithium stearate (0.7%) and polyisobutylene (1.9% Paratac) to produce a MacMichael viscosity of about 25 was added to a 150 SUS (at 100°F.) hydrorefined naphthenic lube (aniline point 162) to which there was also added 1.3% of 40% chlorinated paraffin (Chlorfin 40), to improve load carryability of the oil, 0.4 of tertiarybutyl paracresol and 2 ppm of a silicone antifoam. This lithium soap thickened textile lubricant cannot be made with a paraffinic base oil of the same viscosity since the paraffinic oil is not sufficiently compatible with soap to permit attainment of the desired MacMichael viscosity. Unhydrorefined naphthenic oil cannot be used in this oil because it causes discoloration and damage to textiles.

The soap thickened, antileak hydraulic oils described herein can be used as a functional fluid in energy absorber devices, such as those which can reduce the body and bumper damage caused by automotive collisions (e.g., see Publications 710536, 710537 and 710540 of the Society of Automotive Engineers; mid year meeting, Montreal, Quebec, Canada on June 7-11, 1971. In such a combination the base oil should have an aniline point of about 200°F. when the seals are of silicone rubber.

An aluminum "complex" soap concentrate, which is useful in the present invention, can be made as follows (all parts are by weight):

Dissolve 0.7 parts benzoic acid in 500 parts of bright stock (or other high viscosity lube) at 220°F.

Dissolve 13 parts stearic acid in 450 parts of paraffinic bright stock (or other high viscosity lube) at 200°F.

Add Agrashell Kolate, 3 parts, to the stearic acid in oil, mix and stir (e.g., about 8 minutes).

Add the benzoic acid in oil to the stearic-acid-oil-Kolate, heat with stirring, to 400°F. then cool, with stirring to 220°F.

The concentrate is especially useful at levels which impart 0.1-1% Al complex soap to the final hydraulic oil composition.

Agrashell Kolate is a reactive oxoaluminum compound for making complex aluminum soaps and greases.

TABLE I

| Polymeric Type Antileak Hydraulic Oil |                                        |             |                   |                        |
|---------------------------------------|----------------------------------------|-------------|-------------------|------------------------|
| Lubricant Properties                  |                                        | ASTM Method | R&O Hydraulic Oil | Antileak Hydraulic Oil |
| Test                                  |                                        |             |                   |                        |
| 25                                    | Viscosity, SUS/100°F.                  | D2161       | 250               | 242                    |
|                                       | Viscosity, SUS/210°F.                  | D2161       | 50.4              | 45.3                   |
|                                       | Viscosity, Index                       | D2270       | 102               | 34                     |
|                                       | Viscosity, cs/100°F.                   | D445        | 53.9              | 52.1                   |
|                                       | Viscosity, cs/210°F.                   | D445        | 7.4               | 5.82                   |
|                                       | Flash, COC, °F.                        | D92         | 440               | 335                    |
|                                       | Fire, COC, °F.                         | D92         | 495               | 385                    |
|                                       | Pour, °F.                              | D97         | 0                 | -25                    |
|                                       | Color                                  | D1500       | 2.0               | 2.25                   |
|                                       | Gravity, °API                          | D287        | 31.2              | 21.2                   |
|                                       | TAN, mgKOH/g                           | D664        | 0.07              | 0.0                    |
|                                       | Copper Strip, class                    | D130        | 1                 | 1                      |
|                                       | Aniline Point, °F.                     | D611        | 230               | 152                    |
| 30                                    | Demulsibility/130°F. Separation, min.  | D1401       | 10                | 20                     |
|                                       | Foam, Tendency/Stability               | D892        |                   |                        |
|                                       | Sequence I, ml                         |             | 20/0              | 5/0                    |
|                                       | Sequence II, ml                        |             | 20/0 25/0         |                        |
|                                       | Sequence III, ml                       |             | 20/0              | 20/0                   |
| 35                                    | Rust, Syn Sea Water                    | D665B       | Pass              | Pass                   |
|                                       | Oxidation Stability, hr <sup>(1)</sup> | D943        | 1,300             | 1,250                  |
|                                       | Leak Resistance                        |             | —                 |                        |
|                                       | Gms Leaked                             |             | 110               | 65                     |
|                                       | Reduction, %                           |             | —                 | 41                     |
| 40                                    |                                        |             |                   |                        |

(1) To 2.0 TAN end point.

TABLE II

| Plant Trial Data.                                             | Consumption, Gallons in |                        |          |
|---------------------------------------------------------------|-------------------------|------------------------|----------|
|                                                               | R&O Hydraulic Oil       | Antileak Hydraulic Oil |          |
| 1 Plant Trial<br>Per Broach per week* at                      |                         |                        |          |
| Division A                                                    | 5.7                     | 3.1                    | 46       |
| Division B                                                    | 23.1                    | 2.7                    | 88       |
| Division C. 10.0                                              | 5.0                     | 50                     |          |
| 2 Plant Trial<br>Total plant usage**<br>Per unit manufactured | 3,131,667<br>.98        | 2,242,766<br>.75       | 28<br>24 |

\* month duration

11  
TABLE III

| Type Equipment       | Polymeric Antileak Hydraulic Oil                               |     |
|----------------------|----------------------------------------------------------------|-----|
|                      | #2 Plant Trial Leakage Comparison in<br>Most Critical Machines |     |
|                      | Average Weekly Consumption, Gallons                            |     |
| Broach               | 108                                                            | 57  |
| Automated Drill line | 41                                                             | 33  |
| Mill                 | 12                                                             | 19  |
| Drill                | 217                                                            | 155 |
| Gear Cutter          | 140                                                            | 112 |
| Drill                | 198                                                            | 35  |
| Lathe                | 217                                                            | 178 |
| Broach               | 32                                                             | 28  |
| Gear Cutter          | 102                                                            | 57  |
| Grinder              | 28                                                             | 6   |
| Drill                | 23                                                             | 16  |
| Lathe                | 66                                                             | 25  |
| Total                | 1,184                                                          | 721 |
| % Reduction          |                                                                | 39  |

TABLE IV

| Gel Type Antileak Hydraulic Oil Lubricant Properties |             |                   |                        |
|------------------------------------------------------|-------------|-------------------|------------------------|
| Test                                                 | ASTM Method | R&O Hydraulic Oil | Antileak Hydraulic Oil |
| Viscosity, SUS/100°F.                                | D2161       | 250               | 258                    |
| Viscosity, SUS/210°F.                                | D2161       | 50.4              | 45.5                   |
| Viscosity, Index                                     | D2270       | 102               | 23                     |
| Viscosity, cs/100°F.                                 | D445        | 53.9              | 55.6                   |
| Viscosity, cs/210°F.                                 | D445        | 7.4               | 5.9                    |
| Flash, COC, °F.                                      | D92         | 440               | 350                    |
| Fire, COC, °F.                                       | D92         | 495               | 390                    |
| Pour, °F.                                            | D97         | 0                 | -40                    |
| Color                                                | D1500       | 2.0               | 2.5                    |
| Gravity, °API                                        | D287        | 31.2              | 22.1                   |
| TAN, mgKOH/g                                         | D664        | 0.07              | 0.0                    |
| Copper Strip, class                                  | D130        | 1                 | 1                      |
| Aniline Point, °F.                                   | D611        | 230               | 160                    |
| Demulsibility/130°F.                                 | D1401       |                   |                        |
| Separation, min.                                     |             | 10                | 25                     |
| Foam, Tendency/Stability                             | D892        |                   |                        |
| Sequence I, ml                                       |             | 20/0              | 5/0                    |
| Sequence II, ml                                      |             | 20/0              | 25/0                   |
| Sequence III, ml                                     |             | 20/0              | 5/0                    |
| Rust, Syn Sea Water                                  | D665B       | Pass              | Pass                   |
| Oxidation Stability, hr <sup>(1)</sup>               | D943        | 1,300             | 900                    |
| Leak Resistance                                      |             |                   |                        |
| Gms Leaked                                           |             | 110               | 20                     |
| Reduction, %                                         |             | —                 | 82                     |

(1) To 2.0 TAN end point.

12  
TABLE VI

| 5 | Properties of Hydrocracked Oils* |            |                |                   |                         |
|---|----------------------------------|------------|----------------|-------------------|-------------------------|
|   | Viscosity<br>(SUS, 100°F.)       | ASTM<br>VI | Gravity<br>API | Wt.%<br>Aromatics | Aniline<br>Point<br>°F. |
|   | 100                              | 103        | 34.2           | 12                | 220                     |
|   | 200                              | 107        | 33.3           | 11                | 235                     |
|   | 500                              | 107        | 31.5           | 13                | 250                     |

10 \* All oils dewaxed to a 0°F. pour point by chilling in a solvent.

- 15 The invention claimed is:
1. A soap thickened antileak hydraulic oil comprising an effective amount for thickening of a lithium soap of a fatty acid having 12-22 carbon atoms or an aluminum soap of said acid, and a hydrocarbon base oil having a viscosity in the range of 80-3000 SUS at 100°F said base oil consisting essentially of a blend of at least one hydrorefined naphthenic oil and at least one hydrocracked paraffinic oil, each said oil having a viscosity in the range of 40-12,000 SUS at 100°F.
  - 20 2. Hydraulic oil according to claim 1 and wherein said hydrorefined naphthenic oil contains less than 80 ppm of basic nitrogen and has a viscosity-gravity constant in the range of 0.840-0.899.
  - 25 3. Hydraulic oil according to claim 1 and wherein said soap is lithium stearate.
  - 30 4. Hydraulic oil according to claim 1 and containing in addition a zinc dialkyl dithiophosphate antiwear agent.
  - 35 5. Hydraulic oil according to claim 4 and wherein said hydraulic oil contains in the range of 0.1-1% lithium stearate, in the range of 0.02-2% neutral barium petroleum sulfonate and in the range of 0.1-5% zinc dialkyl dithiophosphate.
  - 40 6. Hydraulic oil according to claim 3 and containing in the range of 0.3-2% zinc dialkyl dithiophosphate antiwear agent.
  - 45 7. Hydraulic oil according to claim 1 and wherein said base oil has a viscosity at 100°F. in the range of 150-350 SUS.
  8. Hydraulic oil according to claim 7 and containing in the range of 0.1-1% lithium stearate.
  9. Hydraulic oil according to claim 1 wherein said base oil consists of a blend of at least one hydrorefined

TABLE V

| Gel Type Antileak Hydraulic Oil Plant Trial Data |                  |                    |                |
|--------------------------------------------------|------------------|--------------------|----------------|
| Equipment                                        | Horizontal Press | Vertical Press     | Vertical Press |
| Type                                             | Horizontal Press | Vertical Press     | Vertical Press |
| Ram Diameter                                     | 12"              | 22"                | 36"            |
| Oil Capacity                                     | 150 gal          | 200 gal            | 300 gal        |
| Operation                                        |                  |                    |                |
| Pressure                                         | 1500 psi         | 1000 psi. 1500 psi |                |
| Temperature                                      | Ambient          | 150°F              | 125°F          |
| Duration                                         | 880 hr           | 1944 hr            | 1400 hr        |
| Leakage                                          |                  |                    |                |
| R&O Hydraulic Oil                                | 75-100 gal/wk    | 50 gal/wk          | 125 gal/wk     |
| Hydraulic Oil                                    | 35-40 gal/wk     | 7 gal/wk           | 50 gal/wk      |
| Reduction, %                                     | 55-60            | 85                 | 60             |

13

naphthenic oil and at least one hydrocracked paraffinic oil.

10. Hydraulic oil according to claim 1 wherein said base oil contains less than 80 ppm of basic nitrogen.

11. Hydraulic oil according to claim 1 wherein said base oil has an aniline point in the range of 150°-170°F.

12. Hydraulic oil according to claim 1 and having an aniline point in the range of 195°-215°F. said hydraulic oil being suitable for use in contact with a silicone rubber.

13. Hydraulic oil according to claim 1 and having an aniline point of about 200°F.

14. Hydraulic oil according to claim 1 and wherein said soap is selected from stearates, palmitates, tallates, laurates, oleates and mixtures thereof.

15. Hydraulic oil according to claim 1 wherein said oil contains in addition a member selected from low nitrogen content paraffinic distillate, low nitrogen content paraffinic solvent raffinate oil, hydrorefined paraffinic distillate, hydrorefined paraffinic raffinate, polycyclic aromatic concentrate, unhydrorefined naphthenic distillate, and naphthenic acid-free naphthenic distillate.

14

16. A polymer thickened antileak hydraulic oil comprising a polybutene having a molecular weight higher than several hundred thousand in amount effective to thicken the oil and a base oil consisting essentially of a blend of hydrorefined naphthenic oil and hydrocracked paraffinic oil.

17. A soap thickened antileak hydraulic oil comprising an effective amount, for thickening, of a lithium soap of a fatty acid having 12-22 carbon atoms or of an aluminum soap of said acid, and a hydrocarbon base oil having a viscosity in the range of 80-3000 SUS at 100°F., said base oil consisting essentially of a hydrorefined naphthenic oil or a blend of two or more hydrorefined naphthenic oils having a viscosity in the range of 40-12,000 SUS at 100°F., at least one said hydrorefined naphthenic oil containing less than 80 ppm of basic nitrogen and having a viscosity-gravity constant in the range of 0.840-0.899.

18. Hydraulic oil according to claim 17 wherein said base oil is a blend of at least two hydrorefined naphthenic oils.

\* \* \* \* \*

25

30

35

40

45

50

55

60

65